

# UNITED STATES PATENT OFFICE.

NICKOLAUS A. PAPADIMITROPOULUS, OF FITZGERALD, GEORGIA.

## COMPOUND FUEL.

1,123,581.

Specification of Letters Patent.

Patented Jan. 5, 1915.

No Drawing.

Application filed March 27, 1914. Serial No. 327,715.

*To all whom it may concern:*

Be it known that I, NICKOLAUS A. PAPADIMITROPOULUS, a subject of the King of Greece, residing at Fitzgerald, in the county of Ben Hill and State of Georgia, have invented certain new and useful Improvements in Compound Fuels; and I do hereby declare the following to be a full, clear, and exact description of the invention, such as will enable others skilled in the art to which it appertains to make and use the same.

This invention relates to compound fuels and the processes of making the same, and the principal object of the invention is to provide a compound fuel having hydro-carbon base which can be entirely consumed without leaving any residue ashes, which will produce but little smoke, which shall be comparatively light in weight, and easily packed within a small compass in briquettes or blocks, and which will produce more heat units per pound than coal or other natural fuels.

Another object of the invention is to produce a compound fuel for use with locomotive boilers or for use on steamships or for stationary boilers and furnaces which shall be comparatively light in weight, which will not produce cinders nor ashes when burned, which will produce a high degree of heat for a great length of time, which can be packed in a small compass and which can be produced at comparatively low cost.

In carrying out the invention, the following ingredients and proportions may be utilized:

|                                    |           |    |
|------------------------------------|-----------|----|
| Kerosene oil or crude hydro-carbon | 16 parts. | 40 |
| Paraffin                           | 5 parts.  |    |
| Ordinary laundry soap              | 3 parts.  |    |
| Table salt, pulverized             | 1 part.   |    |

The paraffin, soap, and salt are dissolved in sufficient hot water for mixing them thoroughly together and dissolving the paraffin and soap, and while still hot, the kerosene oil or hydro-carbon material is added and the whole thoroughly mixed together, after which it is poured out into molds of the required size and permitted to set and harden. The proportions of the various ingredients may be changed without materially effecting the combustible quality of the fuel.

What is claimed is:—

A compound fuel consisting of kerosene oil, sixteen (16) parts, paraffin, five (5) parts, common laundry soap, three (3) parts, table salt, one (1) part, and sufficient water to make a plastic compound to be molded into blocks.

In testimony whereof I have affixed my signature in presence of two witnesses.

NICKOLAUS A. PAPADIMITROPOULUS.

Witnesses:

A. L. MOORE,  
CHARLES A. MOORE.